

April 24, 1962

A. PIERROT ET AL

3,031,405

FERROMAGNETIC MATERIALS HAVING A RECTANGULAR HYSTERESIS CYCLE

Filed Dec. 9, 1957

7 Sheets-Sheet 1



Inventor  
A. Pierrot - Y. Lescroel

By *John M. Calmefle*  
Attorney

April 24, 1962

A. PIERROT ET AL

3,031,405

FERROMAGNETIC MATERIALS HAVING A RECTANGULAR HYSTERESIS CYCLE

Filed Dec. 9, 1957

7 Sheets-Sheet 2



Inventor  
A. Pierrot - V. Lescroel

By *John M. Calmapple*  
Attorney

April 24, 1962

A. PIERROT ET AL

3,031,405

FERROMAGNETIC MATERIALS HAVING A RECTANGULAR HYSTERESIS CYCLE

Filed Dec. 9, 1957

7 Sheets-Sheet 3



Inventor  
A.Pierrot - Y.Lescroel

By *John M. Calmefield*  
Attorney

April 24, 1962

A. PIERROT ET AL

3,031,405

FERROMAGNETIC MATERIALS HAVING A RECTANGULAR HYSTERESIS CYCLE

Filed Dec. 9, 1957

7 Sheets-Sheet 4

Fig. 9.



Fig. 10



Fig. 11.



Inventor  
A. Pierrot - Y. Lescroel

By *John M. Calm after*  
Attorney

April 24, 1962

A. PIERROT ET AL

3,031,405

FERROMAGNETIC MATERIALS HAVING A RECTANGULAR HYSTERESIS CYCLE

Filed Dec. 9, 1957

7 Sheets-Sheet 5



Inventor  
A.Pierrot - Y.Lescroel

By *John M. Calmefle*  
Attorney

April 24, 1962

A. PIERROT ET AL

3,031,405

FERROMAGNETIC MATERIALS HAVING A RECTANGULAR HYSTERESIS CYCLE

Filed Dec. 9, 1957

7 Sheets-Sheet 6



Inventor  
A.Pierrot - Y.Lescroel

By John M. Calmapple  
Attorney

April 24, 1962

A. PIERROT ET AL

3,031,405

FERROMAGNETIC MATERIALS HAVING A RECTANGULAR HYSTERESIS CYCLE

Filed Dec. 9, 1957

7 Sheets-Sheet 7

FIG. 17.



FIG. 18.



FIG. 18A

FIG. 17A

FIG. 19.



Inventor

A. Pierrot - Y. Lescroel

By *John M. Calmeyelle*

Attorney

1

3,031,405

## FERROMAGNETIC MATERIALS HAVING A RECTANGULAR HYSTERESIS CYCLE

André Pierrot and Yves Lescroel, Conflans Sainte-Honorine, France, assignors to Lignes Télégraphiques et Téléphoniques, Paris, France, a French company  
Filed Dec. 9, 1957, Ser. No. 701,612  
Claims priority, application France Dec. 14, 1956  
3 Claims. (Cl. 252—62.5)

The present invention relates to ferromagnetic materials of the ferrite type, having substantially rectangular hysteresis cycles and methods of manufacturing such materials. Materials of this kind can be employed in magnetic recording devices known as "memory devices," magnetic control members, magnetic amplifiers, etc. In such applications these materials are used in the form of cores, usually of toroidal shape or at least of closed shape, without air-gap.

Materials with a hysteresis cycle of rectangular form were already known, particularly alloys of iron or of iron and silicon, of which the magnetic properties are most frequently rendered anisotropic either by cold rolling or by heat treatment under a magnetising field. These materials, generally speaking, have high magnetic moments at saturation and low coercive fields.

The great drawback of these metallic materials, despite their usually high magnetic moment at saturation, is the low value of their resistivity, which leads to considerable eddy current losses. These high losses result in an increase of the response time and a deformation of the hysteresis cycle, which then loses its character of rectangularity as soon as the frequency increases. If it be desired to employ these cores at frequencies of several megacycles per second, they must be obtained in very thin form, of the order of a few microns, and their price immediately becomes prohibitive.

Before explaining the present invention, some notations and definitions are given of the magnetic magnitudes which will be employed in the following, and it is specified that the values of the magnetic moment in gauss, is the product by  $4\pi$  of the value of the magnetic moment in electromagnetic c.g.s. units.

A substantially rectangular hysteresis cycle, plotted for a magnetic field practically reaching saturation, is defined by the following coefficients:

$I_s$  = moment at saturation, gausses,

$I_r$  = remanent moment corresponding to the cycle at saturation, in gausses,

$H_c$  = coercive field corresponding to the cycle at saturation, in oersteds,

$\beta_r$  = ratio of the remanent moment to the moment at saturation.

Moreover, the following coefficients correspond to one work cycle, going from a positive maximum magnetising field ( $+H_m$ ) to the maximum negative field ( $-H_m$ ):

$I_m$  = moment corresponding to the field  $H_m$  in gausses

$B_m$  = induction corresponding to the field  $H_m$  in gausses,

$B_{rm}$  = remanent induction, in gausses,

$B_{dm}$  = final value of the induction when the magnetising field is made to pass from a value  $H_m$  comprised between  $H_{cm}$  and  $2H_{cm}$  to the value  $(-\frac{H_m}{2})$ ,

$H_{cm}$  = coercive field, in oersted,

$\beta_m$  =  $\frac{B_{rm}}{B_m}$  or "coefficient of rectangularity,"

$R_m$  =  $\frac{B_{dm}}{B_m}$  or "ratio of rectangularity,"

2

It is also possible, in certain cases, to evaluate the slopes of the substantially vertical and horizontal sides of the hysteresis cycle.

The quantities:

$$P_h = \left( \frac{\Delta I}{\Delta H} \right)_h$$

and

$$P_v = \left( \frac{\Delta I}{\Delta H} \right)_v$$

in which  $\Delta I$  and  $\Delta H$  are small variations of the moment and of the magnetising field in the vicinity of a given point, and are respectively defined in the vicinity of the intersection of the curve representing the hysteresis cycle with the axes of coordinates,  $P_h$  corresponding to a zero field and  $P_v$  to a zero moment.

For an ideal rectangular cycle, the values of  $P_h$  and  $P_v$  would tend respectively towards zero and towards infinity.

The permeability  $\mu$  is defined as the initial permeability in the demagnetised state.

The coefficients of magnetic losses employed are the Jordan coefficients; in only considering the contribution of the eddy current losses to the loss resistance  $R_p$ , therefore, the coefficient of eddy current losses is defined by the Jordan relation:

$$F_n = \frac{R_p}{L} \left( \frac{800}{f} \right)^2$$

$R_p$  being the loss resistance, expressed in ohms,  $f$  being the frequency, expressed in cycles per second,  $L$  being the inductance, expressed in henrys.

The coefficient of eddy current losses  $F_n$ , expressed in ohms per henry, for the frequency  $f=800$  c./s., is measured between 100 and 200 kc./s., for a field of 2 milliorsteds and at a temperature of about  $20^\circ$  C., for magnetic circuits of which the cross-section is about 0.3 cm.

The Curie point  $\theta_c$ , in the following will be, by convention, the temperature expressed in degrees centigrade, above which the material is no longer ferromagnetic.

The magnetostrictive effects can be characterised by the value of the coefficient of magnetostriction at saturation  $\lambda_s$ , obtained by extrapolating for the demagnetised state the relative curve of variation

$$\frac{\Delta l}{l}$$

in the direction of the applied field, of the length  $l$  of the sample plotted for very high fields.

Another important characteristic is the variation of  $B_m$  or of  $I_s$  as a function of the temperature; it is defined by a coefficient of variation of induction in percent per degree:

$$\alpha_B = \frac{1}{B_m} \cdot \frac{\Delta B_m}{\Delta t} \cdot 10^2$$

$B_m$  being the value of the induction at  $20^\circ$  C.

$\Delta B_m$  being the variation of induction between  $20^\circ$  and  $80^\circ$  C.,

$\Delta t$  being the corresponding difference of temperature, that is to say, in the present case  $\Delta t=60^\circ$  C.

The induction  $B_m$  corresponds to a particular field  $H_m$  which is clearly higher than  $H_c$ .

The "response time" is defined by considering two windings with negligible time constants placed on a core made of the magnetic material concerned, this core is

subjected to the magnetising field  $H_m$  comprised between  $H_{cm}$  and  $2H_{cm}$ , then to the field

$$\left( \frac{-H_m}{2} \right)$$

then there is applied to one of the windings a current pulse of which the rising time is very short. Two windings are used one of which  $N_1$  consists of three turns and the other  $N_2$  of a single turn. The dimensions of the core on which these windings are placed are: external diameter 2 mm.; internal diameter 1.2 mm.; height 0.88 mm. A series of five impulses is then passed through the winding  $N_1$  as follows: a positive impulse of  $I$ ; a negative impulse  $I$ ; two positive impulses value  $I/2$ ; a negative impulse of  $I$ . The interval between the pulses is 50 microseconds; the rise time of each impulse being 0.3 microsecond. The response given in winding  $N_2$  to the second impulse is then considered. The response time  $\tau$  is taken as the time, in microseconds, required for the voltage produced in winding  $N_2$ , starting from one tenth of the maximum to pass through the maximum and return to 10% of the value of this maximum.

The object of the invention is to produce magnetic materials of the ferrite type having on the one hand, substantially rectangular hysteresis cycles, and on the other hand high resistivities  $\rho$  at least equal to  $10^3$  ohms-centimetre.

The rectangularity of the cycle is obtained by starting with materials of the ferrite type with negative coefficients of magnetostriction which are subjected to stresses. According to one form of the invention these materials are subjected to natural stresses obtained by a heat treatment by means of which a considerable linear shrinkage is produced, of at least 8% and which may go up to 30%. By this means a cycle of rectangularity having a coefficient of rectangularity  $\beta_m$  at least equal to 0.8 may be obtained.

Further according to the invention magnetic materials of the above kind in addition to the natural stresses obtained during heat treatment may be subjected in the form of the finished core to external artificial mechanical stresses. It has been verified that in this way the rectangularity of the cycle is further improved; a coefficient of rectangularity  $\beta_m$  at least equal to 0.95 is obtained, and, what is particularly remarkable, a rectangularity ratio  $R_m$  greater than 0.9 is obtained, a value unequalled hitherto.

The said external artificial mechanical stresses can be realised by known processes, hydraulic, the core being placed in a receptacle into which oil or water is forced under pressure, or mechanical,

(a) The core is surrounded by a band of rubber or the like, the whole is placed in a clamping means to compress the band

(b) The exterior surface of the core is covered with enamel, which is cured

(c) The wound core is embedded in a resin which, after compression or preferably after polymerisation, exercises a considerable stress on cooling.

All forms of cores presenting a closed magnetic circuit without an air gap may be thus treated.

This artificial mechanical stress is applied to the core after heat treatment and the applied stress is maintained during use.

In view of their high resistivity, these materials have negligible eddy-current losses which enable them to be used at high frequency with low response time ( $\tau \leq 10$  microseconds).

The materials in accordance with the invention have coefficients of rectangularity  $\beta_m$  and ratios of rectangularity at least equal to the values indicated above. In addition they have inductions at saturation ( $\beta_s$ ) of the order of 1,500 to 4,500 gauss at 20° C. coefficients of variation

of induction as a function of the temperature  $\alpha_B$  at most equal to 0.5 and Curie points  $\theta_c$  higher than 200° C.

The ferrromagnetic materials which are the object of the present invention are ferrromagnetic materials of the ferrite type, with substantially rectangular hysteresis cycle, manufactured by compressing a homogeneous mixture of fine powders of metallic oxides under a pressure of from 0.5 to 15 tons per square centimetre and by subjecting the cores obtained from the mixture to a heat treatment consisting of heating to a temperature comprised between 900° C. to 1,300° C. in oxygen, followed by cooling for about 15 hours, the said mixture consisting of ferric oxide and optionally oxides of trivalent metals of the group comprising aluminum and chromium, oxides of at least two bivalent metals of the group containing nickel and copper, and optionally oxides of bivalent metals of the group comprising zinc and cadmium, characterised in this, that in the said mixture the sum of the molecular percentages of the oxides of the trivalent metals is comprised between 47 and 50, the sum of the molecular percentages of the oxides of the trivalent metals, other than iron, being less than or equal to 2, the sum of the molecular percentages of the oxides of the bivalent metals of the group comprising nickel and copper being comprised between 25 and 53; the percentage of the copper oxide being comprised between 3 and 15 and the sum of the molecular percentages of the oxides of bivalent metals of the group comprising zinc and cadmium being at most equal to 25.

30 The invention will be described in more detail in the following for ferrites of which the starting compositions satisfy the formula:

$$x\text{Fe}_2\text{O}_3, u\text{NiO}, v\text{CuO}, s\text{ZnO}, y\text{T}_2\text{O}_3$$

35 in which  $T$  may be one or more trivalent metals such as aluminum and chromium, in which  $x$ ,  $y$ ,  $u$ ,  $v$  and  $s$  designate the molecular percentages satisfying the following relations:

$$x+y+u+v+s=100,$$

$$47 \leq x+y \leq 50,$$

$$0 \leq y \leq 2,$$

$$35 \leq u+v \leq 53,$$

$$3 \leq v \leq 15$$

and

$$0 \leq s \leq 15.$$

In the whole of the rest of the description the compositions indicated are the starting compositions before grinding. The increase of the iron content due to the wear of the grinder, being for an average mill, about 0.8 molecule of  $\text{Fe}_2\text{O}_3$  percent molecules of ground material; the given percentages of  $\text{Fe}_2\text{O}_3$  after grinding must be increased by this quantity; it would be necessary to make corrections if a mill were used which wore out more slowly or more quickly.

60 It is well-known that the magnetostriction of a mixed ferrite material depends upon the magnetostriction of each of the ferrites of which it is composed. Of all the ferrites, only the ferrite of iron or magnetic oxide of iron  $\text{FeO} \cdot \text{Fe}_2\text{O}_3$  (that is  $\text{Fe}_3\text{O}_4$ ) shows a positive coefficient of magnetostriction.

In accordance with the invention it is necessary in order to obtain a material with substantially rectangular hysteresis cycle to form a ferrite having little or no bivalent iron. Now the maximum molecular percentage of the iron oxide being equal to 50 there will only be very little bivalent iron or even none at all and the conditions required for the material to have a negative coefficient of magnetostriction are, therefore, well satisfied.

70 The invention will be described in more detail in the following with reference to the attached drawings:

FIG. 1 represents a substantially rectangular hysteresis cycle;

FIG. 2 represents a triangular diagram indicating com-

positions of materials in accordance with the invention.

FIG. 3 represents curves of variation of induction  $B_m$ , as a function of the molecular percentage of  $Fe_2O_3$ ;

FIG. 4 represents curves of variation of the coefficient of rectangularity  $\beta_m$  as a function of the molecular percentage of  $Fe_2O_3$ ;

FIG. 5 represents curves of variation of induction  $B_m$ , as a function of the molecular percentage of  $Al_2O_3$  or of  $Cr_2O_3$  in a defined compound;

FIG. 6 represents curves of variation of the coefficient of rectangularity  $\beta_m$  as a function of molecular percentage of  $Al_2O_3$  or  $Cr_2O_3$ , in a defined compound.

FIG. 7 represents the variation of the induction  $B_m$  as a function of  $H_m$  for a defined compound;

FIG. 8 represents the variation of  $R_m$ , and of  $\beta_m$  as a function of  $H_m$  for a defined compound;

FIG. 9 represents the variation of the induction  $B_m$  as a function of the temperature for two defined compounds;

FIG. 10 represents the variations of the coercive field  $H_{cm}$ , as a function of the temperature for two defined compounds;

FIG. 11 represents the variation of the ratio of rectangularity  $\beta_m$ , as a function of the temperature for two defined compounds;

FIGS. 12 to 16 represent hysteresis cycles of material according to the invention.

FIGS. 17, 17a and 18, 18a each represent, in horizontal and vertical section a core enveloped in a polyester resin;

FIG. 19 represents, for different fields, hysteresis cycles for a magnetic core not enveloped and for the same core enveloped in polyester resin.

In FIG. 1 which represents a rectangular hysteresis cycle corresponding to a field  $H_m$ , are indicated the induction  $B_m=OR$ , the remanent induction  $B_{rm}=OP$ , the induction  $B_{dm}=OS$  corresponding to the field

$$\left(-\frac{H_m}{2}\right)$$

as also the coercive field  $H_{cm}$ .

The "coefficient of rectangularity" is

$$\beta_m = \frac{B_{rm}}{B_m} = \frac{OP}{OR}$$

for the "ratio of rectangularity";

$$R_m = \frac{B_{dm}}{B_m} = \frac{OS}{OR}$$

and, for the ratio  $K_m$ :

$$K_m = \frac{B_{rm} + B_m}{B_{rm} - B_{dm}} \frac{OP + OT}{OP - OS}$$

FIG. 2 represents a triangular diagram corresponding to a material according to the invention, of which the three components are: the sum of the molecular percentages of the oxides of trivalent metals  $Fe_2O_3$ ,  $Cr_2O_3$ ,  $Al_2O_3$ , the sum of the molecular percentages of the oxides of bivalent metals  $NiO$  and  $CuO$  and the sum of the molecular percentages of bivalent metals  $ZnO$  and  $CdO$ . The figurative point of the composition with rectangular hysteresis cycle, in accordance with the invention, must be located inside the hatched zone A, B, C, D, which appears in the form of an elongated parallelogram. Above the limit C-B there may again be compositions satisfying the condition of rectangularity  $\beta_m \geq 0.80$  but the Curie point  $\theta_c$  becomes lower as the molecular content of  $ZnO$  increases and the condition  $\alpha_B < 0.50$  can no longer be guaranteed.

In all the following, the characteristics of the hysteresis cycle have been marked on the flux-meter on toroidal cores of the approximate dimensions:

External diameter=34.3 mm.,

Internal diameter=27.3 mm., and

Height=11 mm.

wound with 100 turns of copper wire 0.30 mm. in diameter for the "field" winding and 200 turns of copper wire 0.15 mm. in diameter for the "induction" windings.

FIG. 3 shows curves of variation of induction  $B_m$ , marked at  $H_m=10$  oersteds as a function of the molecular percentage of  $Fe_2O_3$ . In all these compounds, the molecular percentage of  $CuO$  was 5, and each curve corresponds to a family of compounds of constant molecular content of  $ZnO$ ; these molecular percentages of  $ZnO$  corresponding to the four curves are respectively 0, 5, 10 and 15. All these compounds have been treated under the same conditions; in particular they have been sintered at 1200° C. for two hours in oxygen. It will be noted that when the molecular percentage of  $ZnO$  increases, the maximum of  $B_m$  is shifted to the right, that is to say, towards higher molecular percentages of  $Fe_2O_3$  and that this maximum reaches a higher value.

In FIG. 4, curves of variation of the coefficient of rectangularity  $\beta_m$ , for  $H_m=10$  oersteds are shown as a function of the molecular percentage of  $Fe_2O_3$ . All the compounds compared are the same as those of which the properties are represented in FIG. 3 and they are grouped in the same manner. It will be noted that the maximum of  $\beta_m$  occurs approximately, for the same molecular percentage of  $Fe_2O_3$  as that which gives the maximum of  $\beta_m$ . The value of the maximum of  $\beta_m$  is adjacent to 0.90.

FIG. 5 shows the variation of the induction  $B_m$ , marked at 10 oersteds, for a family of compounds:

(49-y)  $Fe_2O_3$ ,  $yT_2O_3$ , 36NiO, 5CuO, 10ZnO as a function of  $y$ ; the curve  $C_1$  is relative to the case in which T represents aluminum and the curve  $C_2$  is relative to the case in which T represents chromium. It is clear that the substitution of molecules of  $Al_2O_3$  or of  $Cr_2O_3$  for an equal number of  $Fe_2O_3$  molecules in the compound:

$$49Fe_2O_3, 36NiO, 5CuO, 10ZnO$$

has the effect of reducing the maximum induction.

40 In FIG. 6 is represented the variation of the coefficient of rectangularity  $\beta_m$ , marked at 10 oersteds, for the same family of compounds as that corresponding to FIG. 5, as a function of the molecular percentage of  $Al_2O_3$  (curve  $C_3$ ) or as a function of the molecular percentage of  $Cr_2O_3$  (curve  $C_4$ ). All these compounds have been treated under the same conditions and in particular have been sintered at 1,200° C. for two hours in oxygen. The coefficient for rectangularity  $\beta_m$  decreases slightly when the molecular content of  $Cr_2O_3$  or of  $Al_2O_3$  increases. It 50 will be seen moreover, that in both cases the influence of  $Cr_2O_3$  is more marked than that of  $Al_2O_3$ .

It is possible with reference to FIGS. 7 and 8 to examine the influence of the work field  $H_m$  on the characteristics; the results are represented which are obtained 55 on the ferrite composition:

$$49Fe_2O_3, 36NiO, 5CuO, 10ZnO$$

which has been sintered at 1,200° C. for two hours in oxygen.

60 FIG. 7 represents the curve of variation of the induction  $B_m$ , as a function of the field  $H_m$ ; it is in fact the curve of first magnetisation.

FIG. 8 represents the curves of variation of the coefficient of rectangularity  $\beta_m$  and of the ratio of rectangularity  $R_m$  as a function of the field  $H_m$ . It will be seen that  $\beta_m$  increases very rapidly at the start, passes through a slight maximum of the order of 0.93 at 5 oersteds, then decreases very slowly. The curve of  $R_m$  on the other hand, shows a very clear maximum for  $H_m=3.4$  oersteds 70 of which value  $R_m=0.745$ ; the part situated on the right of the maximum is very rapidly decreasing.

The curves of FIG. 8, plotted for an example of predetermined composition, are fairly characteristic and show approximately the same appearance for the other compositions according to the invention; in particular, it will

be seen that the acceptable value of  $R_m$  is obtained for a fairly narrow zone of the field of work; in the present case:  $R_m \geq 0.7$  for 3.2 oersteds  $< H_m < 3.6$  oersteds.

The influence of the temperature will be shown with reference to FIGS. 9, 10 and 11.

In these three figures the curves  $C_5$ ,  $C_7$  and  $C_9$  relate to the ferrite of molecular composition:



and the curves  $C_6$ ,  $C_8$  and  $C_{10}$  relate to the ferrite of molecular composition:



These two compounds have been treated under the same conditions and in particular sintered at 1,200° C. for two hours in an oxygen atmosphere.

FIG. 9 represents the variation of the maximum induction  $B_m$ , marked at  $H_m=10$  oersteds between  $-40^\circ$  C. and  $+100^\circ$  C.; in considering the range from  $20^\circ$  C. to  $80^\circ$  C., it is possible to deduce therefrom:

$\alpha_B = -0.99$  for the compound  $48\text{Fe}_2\text{O}_3, 47\text{NiO}, 5\text{CuO}$  and

$\alpha_B = -0.13$  for the compound  $49\text{Fe}_2\text{O}_3, 36\text{NiO}, 10\text{ZnO}, 5\text{CuO}$ .

FIG. 10 represents the variation of the coercive field  $H_{em}$  for a cycle marked at  $H_m=10$  oersteds between  $-40^\circ$  C. and  $+100^\circ$  C.; in considering the range from  $20^\circ$  C. to  $80^\circ$  C., it is possible to deduce therefrom:

$\alpha H_{em} = -0.02$  for the compound  $48\text{Fe}_2\text{O}_3, 47\text{NiO}, 5\text{CuO}$ , and

$\alpha H_{em} = -0.12$  for the compound  $49\text{Fe}_2\text{O}_3, 36\text{NiO}, 10\text{ZnO}, 5\text{CuO}$ .

FIG. 11 represents the variation of the coefficient of

| Fig.<br>Nos. | Molecular Composition in percent |                         |              |              |              | Magnetic Characteristics |                  |                   |           |       |       |       |       |
|--------------|----------------------------------|-------------------------|--------------|--------------|--------------|--------------------------|------------------|-------------------|-----------|-------|-------|-------|-------|
|              | $\text{Fe}_2\text{O}_3$          | $\text{Al}_2\text{O}_3$ | $\text{NiO}$ | $\text{CuO}$ | $\text{ZnO}$ | $H_m$ ,<br>Oe.           | $B_m$ ,<br>gauss | $H_{em}$ ,<br>Oe. | $\beta_m$ | $R_m$ | $P_h$ | $P_v$ | $F_n$ |
| 12-----      | 48                               | 0                       | 47           | 5            | 0            | 10                       | 2,040            | 3.1               | 0.91      | ----- | 40    | 2,000 | <0.02 |
| 13-----      | 49                               | 0                       | 36           | 5            | 10           | 10                       | 3,100            | 2.5               | 0.89      | ----- | 60    | 5,000 | <0.02 |
| 14-----      | 48                               | 1                       | 36           | 5            | 10           | 3.4                      | 2,340            | 2.2               | 0.905     | 0.745 | 80    | 4,000 | <0.02 |
| 15-----      | 49                               | 0                       | 31           | 5            | 15           | 10                       | 2,790            | 2.8               | 0.88      | ----- | 50    | 2,000 | <0.02 |
| 16-----      | 47.5                             | 0                       | 32.5         | 15           | 5            | 10                       | 3,410            | 1.6               | 0.88      | ----- | 60    | 6,000 | <0.02 |
|              |                                  |                         |              |              |              | 3                        | 2,770            | 1.3               | 0.90      | ----- | 150   | 5,000 | 1.0   |
|              |                                  |                         |              |              |              | 10                       | 2,630            | 2.0               | 0.87      | ----- | 80    | 5,000 |       |

the rectangular  $\beta_m$ , for a cycle marked at  $H_m=10$  oersteds, between  $-40^\circ$  C. and  $+100^\circ$  C.; in considering the range from  $20^\circ$  C. to  $80^\circ$  C., it is possible to deduce therefrom

$\alpha_{\beta_m} = -0.02$  for the compound  $48\text{Fe}_2\text{O}_3, 47\text{NiO}, 5\text{CuO}$ .

$\alpha_{\beta_m} = -0.09$  for the compound  $49\text{Fe}_2\text{O}_3, 36\text{NiO}, 10\text{ZnO}, 5\text{CuO}$ .

It will thus be seen that these materials have coefficients of variation, as a function of the temperature, which are remarkably low in relation to those normally obtained on other types of ferrites, although the addition of a certain percentage of  $\text{ZnO}$  has the effect of increasing these coefficients of variation.

#### METHOD OF MANUFACTURE

##### Composition and Nature of the Oxides Employed

For these mixtures a ferric oxide,  $\text{Fe}_2\text{O}_3$ , copper oxide,  $\text{CuO}$ , nickel oxide,  $\text{NiO}$  are employed and, if necessary, zinc oxide  $\text{ZnO}$ , aluminum oxide  $\text{Al}_2\text{O}_3$  and chromic oxide  $\text{Cr}_2\text{O}_3$ .

These oxides must be pure and the mixture must not contain more than 0.5% impurities.

Silica ( $\text{SiO}_2$ ), barium oxide ( $\text{BaO}$ ), lead oxide ( $\text{PbO}$ ), strontium oxide ( $\text{SrO}$ ), etc., are particularly harmful because these impurities round the angles of the hysteresis cycle.

The content of each of these impurities must be less than 0.05% by weight.

*Grinding*.—The mixture of oxides is ground in an iron mill with steel balls, usually for 12–48 hours, with a weight of distilled water which is substantially double the weight of the mixture of oxides.

*Pressing*.—The influence of the stamping pressure is important. This must be fairly high, so that the moment at saturation of the finished product may be sufficiently high, and on the other hand, fairly low so that the shrinkage during sintering may be great.

10 A pressure of about 5 tons per  $\text{cm}^2$ , corresponding to linear shrinkages of about 15%, has given good results; it is possible to go from 0.5 to 15 tons per  $\text{cm}^2$ .

*Heat treatment*.—In order to obtain the optimum properties, the temperature of annealing must be experimentally adjusted for each composition; generally speaking, the more copper is contained in the ferrite, the more it is necessary to reduce the temperature of annealing; the atmosphere of annealing will be pure oxygen.

#### EXAMPLES

20 FIGS. 12, 13, 14, 15 and 16 represent the hysteresis cycles, plotted in direct current, for a maximum field of 10 oersteds and for another smaller field if necessary. In the latter case, the figure comprises two cycles, that plotted for a field lower than 10 oersteds being inside the other.

The grinding is carried out for 48 hours with an iron ball mill, with a capacity of 16 litres, containing about 3 kg. of mixture, about 6 litres of water and 20 kg. of balls.

30 The annealing is carried out at 1,200° C. for 2 hours in oxygen.

The properties found are summarised in the following Table I.

TABLE I

#### METHODS OF APPLICATION OF THE STRESSES

50 Magnetic materials having the compositions indicated above and subjected to the grinding, pressing and heat treatment described, are then subjected to stresses by one of the known methods given in a non-limitative manner previously. As an example, among others, in order to obtain the compression stresses, use is made of coating the core with a thermosetting resin which permits a considerable shrinkage (10 to 15% after polymerisation) and does not split.

60 As a non-limitative example, we use:

(1) A casting resin which hardens when cold and which is a combination with low viscosity, of non-saturated polyester resins, with monostyrene which can be solidified by polymerisation, with release of heat and considerable shrinkage in the uncharged state.

65 (2) A cobalt accelerator; in principle: cobalt naphthenate or octoate dissolved in a solvent such as those commercially known as white spirit or styrolene.

(3) A catalyst of benzoyl peroxide paste.

70 Ratio of proportions:

|             |       |    |
|-------------|-------|----|
| Resin       | g     | 50 |
| Catalyst    | g     | 5  |
| Accelerator | drops | 2  |

75 The advantages obtained by applying these are ex-

plained hereinafter for the particular case of coating of the magnetic material by polyester resin.

FIGURE 17 shows a core of magnetic material 1 completely coated in polyester resin 2, in which a hole 3 has been arranged to avoid the splitting of the resin in shrinkage. FIGURE 18 represents the same core 1 externally banded by polyester resin 4.

Instead of coating each core individually, it is possible to make a matrix pro forma by coating a perforated plate or by coating a set of cores regularly arranged in a plate with polyester resin.

#### EXAMPLE

FIGURE 19 shows the hysteresis cycles, for different values of the field  $H_m$ , of a core of magnetic material in which the starting composition in molecular percentage is: 48Fe<sub>2</sub>O<sub>3</sub>, 47NiO, 5CuO.

The conditions of sintering are: 2 hours at 1,200° C., in oxygen.

In the whole of the following, the characteristics of the hysteresis cycle have been marked on the fluxmeter, on toroidal cores of approximate dimensions:

External diameter mm 34.7  
Internal diameter mm 27.2  
Height mm 8.8

wound with 200 turns of copper wire of 0.30 mm. diameter for the "field" winding and 200 turns of copper wire of 0.15 mm. diameter for the "inductance" winding.

The cycles *a*, *b* and *c* correspond to the uncoated core and cycles *d*, *e*, *f*, *g* and *h* to the core coated with polyester resin.

The characteristics obtained are given in the following table:

| Core                                          | Curves   | t, ° C. | H <sub>m</sub> , Oe. | B <sub>m</sub> , Gs. | B <sub>rm</sub> , Gs. | H <sub>cm</sub> , Oe. | B <sub>m</sub> | R <sub>m</sub> | K <sub>m</sub> | P <sub>h</sub> | P <sub>v</sub> |
|-----------------------------------------------|----------|---------|----------------------|----------------------|-----------------------|-----------------------|----------------|----------------|----------------|----------------|----------------|
| Not subjected to external mechanical stresses | <i>a</i> | 20      | 10                   | 1.540                | 1.200                 | 4.0                   | 0.78           | -----          | 3.5            | 110            | 470            |
|                                               | <i>b</i> | 20      | 5                    | 567                  | 454                   | 3.1                   | 0.80           | 0.30           | -----          | 60             | 310            |
|                                               | <i>c</i> | 20      | 2                    | 40                   | -----                 | -----                 | -----          | -----          | 4              | 20             | -----          |
|                                               | <i>d</i> | 23      | 10                   | 2.580                | 2.540                 | 2.4                   | 0.98           | -----          | -----          | 4              | -----          |
| Coated with polyester resin                   | <i>e</i> | 23      | 5                    | 2.500                | 2.450                 | 2.4                   | 0.98           | -----          | -----          | 10             | -----          |
|                                               | <i>f</i> | 23      | 3                    | 2.260                | 2.240                 | 2.4                   | 0.98           | 0.98           | 150            | 27             | -----          |
|                                               | <i>g</i> | 23      | 2.7                  | 1.200                | 1.180                 | 2.4                   | 0.98           | 0.92           | 30             | 27             | -----          |
|                                               | <i>h</i> | 23      | 2.4                  | 0                    | -----                 | -----                 | -----          | -----          | 30             | 0              | -----          |

The response time  $\tau$ , for the example under consideration and with the definition and the dimensions previously given, is comprised between 1.0 and 1.5 ms.

Values of the respective intensities:

Complete pulses ma 500  
Partial pulses ma 250

For an uncoated core:

Useful signal (response given by the core after the second pulse), 90 mv.

Interference signal (response given by the core after the last pulse), 42 mv.

Ratio useful signal/interference signal, 2.1.

Response time; between 1 and 1.5 ms.

For a coated core, according to FIGURE 17 or 18, we obtain:

Useful signal, 105 mv.

Signal interference, 30 mv.

Ratio useful-signal/interference, 3.5.

Response time, between 1 and 1.5  $\mu$ s. for the same relative values of current intensity.

What we claim is:

1. Method of manufacturing a unit comprising a ferrite body having a negative coefficient of magnetostriction and a substantially rectangular hysteresis cycle which comprises preparing a homogeneous mixture of oxides according to the formula  $xFe_2O_3yT_2O_3uNiOvCuOsZnO$  in

which T is chosen from the group consisting of aluminum and chromium with the values expressed in molecular percentages,  $x+y$  is between 47 and 50,  $y$  is between 0 and 2,  $v$  is between 3 and 15,  $u+v$  is between 35 and 53 and  $s$  is between 0 and 15,  $x$ ,  $y$ ,  $u$ ,  $v$  and  $s$  being equal to 100, pressing said mixture into core form at a pressure between .05 and 15 tons per square centimeter and heating the pressed core at a temperature between 900° C. and 1300° C. in oxygen followed by cooling for a period of 15 hours.

2. A ferrite having a substantially rectangular hysteresis cycle and a negative coefficient of magnetostriction and made from a starting material having a composition according to the formula:

15



in which T is chosen from the group consisting of aluminum and chromium,  $x+y$  is between 47 and 50,  $y$  is between 0 and 2,  $v$  is between 3 and 15,  $u+v$  is between 35 and 53, and  $s$  is between 0 and 15, all expressed in molecular percentages, the sum of  $x$ ,  $y$ ,  $u$ ,  $v$  and  $s$  being equal to 100, the material being subjected to a pressure of between .05 and 15 tons per square centimeter and heated to a temperature between 900 and 1300° C. in an oxygen atmosphere followed by slow cooling.

3. A core of ferromagnetic material as defined in claim 2, and means to exert artificial mechanical pressure on said core.

30

#### References Cited in the file of this patent

UNITED STATES PATENTS  
2,532,876 Asche et al. Dec. 5, 1950

|           |                 |               |
|-----------|-----------------|---------------|
| 2,551,711 | Snoek et al.    | May 8, 1951   |
| 2,565,861 | Leverenz et al. | Aug. 28, 1951 |
| 2,579,267 | Leverenz et al. | Dec. 18, 1951 |
| 2,601,212 | Polydoroff      | June 12, 1952 |
| 2,685,568 | Wilson          | Aug. 3, 1954  |
| 2,723,239 | Harvey          | Nov. 8, 1955  |
| 2,744,873 | Piekarski       | May 8, 1956   |
| 2,748,099 | Bruner          | May 29, 1956  |
| 2,849,312 | Peterman        | Aug. 26, 1958 |
| 2,962,445 | Pierrot et al.  | Nov. 29, 1960 |

| FOREIGN PATENTS             |
|-----------------------------|
| Great Britain Aug. 17, 1955 |
| Great Britain Apr. 18, 1956 |
| Great Britain July 11, 1956 |
| France Aug. 10, 1955        |
| France May 22, 1956         |

| OTHER REFERENCES                                                                                       |
|--------------------------------------------------------------------------------------------------------|
| Gorter: Philips Research Reports, vol. 9, No. 6, p. 432, December 1954.                                |
| Kordes et al.: Chemical Abstracts, vol. 46, col. 4411, May 25, 1952.                                   |
| Bozorth: Ferromagnetism, Van Nostrand, 1951, pp. 595-712.                                              |
| 70 J. of the Institute of Electrical Engineers, Japan, November 1937, page 5, June 1939, pp. 276, 279. |